

# United States Patent [19]

Luebbecke, Jr. et al.

[11] Patent Number: 4,482,599

[45] Date of Patent: Nov. 13, 1984

- [54] **SUPPORT LAYER FOR ELECTRIC  
DISCHARGE TRANSFER MATERIALS**

[75] Inventors: **Ray H. Luebbe, Jr., Maitland; Mark  
A. Carter, Casselberry, both of Fla.**

[73] Assignee: **Exxon Research & Engineering Co.,  
Florham Park, N.J.**

[21] Appl. No.: **395,103**

[22] Filed: **Jul. 6, 1982**

[51] Int. Cl.<sup>3</sup> ..... **B41M 5/24; G01D 15/06;**  
**G32B 5/16**

[52] U.S. Cl. ..... **428/212; 346/135.1;**  
**428/209; 428/213; 428/457; 428/323**

[58] Field of Search ..... **428/457, 209, 213, 212;**  
**346/135.1**

[56] References Cited

## U.S. PATENT DOCUMENTS

- |           |         |                    |             |
|-----------|---------|--------------------|-------------|
| 4,163,075 | 7/1979  | Nakano et al. .... | 428/469 X   |
| 4,251,612 | 2/1981  | Chu et al. ....    | 430/59      |
| 4,308,314 | 12/1981 | Nakano et al. .... | 346/135.1 X |
| 4,358,474 | 11/1982 | Nakano et al. .... | 428/106 X   |
| 4,390,609 | 6/1983  | Wiedemann ....     | 430/66 X    |

## FOREIGN PATENT DOCUMENTS

- 53-45143 11/1973 Japan ..... 430/67



wherein  $n$  is about 100.

**14 Claims, 1 Drawing Figure**





FIG. I

# SUPPORT LAYER FOR ELECTRIC DISCHARGE TRANSFER MATERIALS

## BACKGROUND OF THE INVENTION

## 1. Field of the Invention

The present invention relates to a composite electro-sensitive transfer material, and more particularly, to a reusable electro-sensitive transfer film.

## 2. Description of the Prior Art

In recent years, various systems have been proposed for the rapid transmission and/or recording of information. One such system is an electric discharge recording system.

The electric discharge recording system is a process which comprises applying an electrical signal of several hundred volts and several watts in the form of an electric voltage, and breaking a semiconductive recording layer on the surface of a recording layer by electric discharge, thereby to form an image on the recording layer or on a substrate superimposed on the recording layer. This process is a "direct imaging" process which does not require processing operations such as development and fixation, and is in widespread use as a simple recording process. For example, the process finds applications in facsimile systems, various measuring instruments, recording meters, record displays in computers, and processing of electrostencil master sheets.

In the electric discharge recording, a discharge recording stylus is directly contacted with the recording surface of an electric discharge recording material. Discharging is performed through the stylus to break the recording layer, and to form an image on the recording surface.

A more recent development is disclosed by Nakano et al in U.S. Pat. No. 4,163,075 and relates to the use of an electrosensitive transfer film. To record with this type of film, it is laid over an untreated sheet of a receiving medium, such as paper, and an electric discharge stylus is moved in a regular pattern across the back of the transfer film. Provision is generally made to ground either one edge or the front surface of the transfer film. When a voltage on the order of 150 to 200 volts is applied to the stylus, current flows through the sheet and matter is caused to be transferred to the receiving sheet, e.g., paper.

The film disclosed by Nakano et al in U.S. Pat. No. 4,163,075, comprises three layers, namely a film support layer and two transfer layers. The support layer is composed of a metal powder-containing resin layer, e.g., electrolytic copper powder having an average diameter of 2 microns dispersed in a vinyl chloride resin.

Numerous disadvantages appear to exist with the use of the products disclosed in the Nakano et al patent. For example, the use of small metal particles in the support layer results in a high cost product affecting the commercial success of the product. A need therefore exists for a transfer sheet exhibiting improved image quality that can be produced at a low cost compared to other commercially available products.

## SUMMARY OF THE INVENTION

It is an object of this invention to provide an electric discharge transfer film which is free from the disadvantages described hereinabove.

Another object of the present invention is to provide an electric discharge transfer film exhibiting improved

image quality, increased stiffness, and increased strength.

A further object of the present invention is to provide an electric discharge transfer film that can be produced in a simple and efficient manner and at a low cost.

According to the present invention, an electric discharge recording material is provided which comprises: (a) an electrically anisotropic support layer having electroconductive particles dispersed in a resin; and (b) at least one thermal or electrothermal transfer layer in the form of a resin layer capable of being broken by electrical discharge and transferred to a record sheet, one of said transfer layers being laminated to said support layer, the improvement wherein said resin in the support layer comprises a phenoxy resin of the formula:



wherein  $n$  is about 100.

Other objects, features and effects of this invention will become more apparent from the following detailed description considered with the drawing wherein:

FIG. 1 is an expanded sectional view of the transfer film of this invention.

## DETAILED DESCRIPTION OF THE INVENTION

According to a preferred embodiment of this invention, the basic film structure, as illustrated in FIG. 1, comprises an electrically anisotropic, electroconductive particle-support layer 2 and two transfer layers, namely layers 4 and 6.

When a graphite-containing resin is employed as layer 2, it generally contains between 5 to 65% and preferably between 15 to 45% by weight graphite based on the weight of the resin. Best results are obtained when the layer contains between 25 and 35% by weight graphite, based on the weight of the resin. The particle diameter of the graphite used in this layer is also critical, Ser. No. 395,102, filed July 6, 1982, entitled ELECTROSENSITIVE TRANSFER FILM the particle size being between 0.1 to 20 microns, and preferably between 0.1-5 microns, with best results being achieved with particles between 0.1 and 1 microns.

The resin which constitutes the resin matrix in which the graphite particles are dispersed is a phenoxy resin of the formula:



wherein  $n$  is about 100

A suitable phenoxy resin is sold by Union Carbide Corporation under the tradename "PKHH". This resin has the following characteristics:

Approximate Molecular Weight 20,000 to 30,000  
 Specific Gravity 1.18  
 Melt Flow (g/10 minutes  
 at 220° C.) 2.5-10

-continued

|                                |                            |
|--------------------------------|----------------------------|
| Ultimate Tensile Strength, psi | 9,000-9,500                |
| Ultimate Tensile Elongation,   | 50-100                     |
| Softening Temperature          | 100° C.                    |
| Moisture Vapor Transmission    | 3.5 gms/mil/24 hrs/100 in. |
| Molecular Structure            |                            |

Generally, the matrix resin preferably has a great ability to bind the electroconductive particles, e.g., graphite or the metal powders disclosed in U.S. Pat. No. 4,163,075 or other useful electroconductive particles that may be used. These resins can be formed into sheets or films having high mechanical strength, flexibility and high stiffness.

It is understood that other resins may be combined with the novel support layer of the present invention. Suitable resins that can be used in this invention are thermoplastic resins such as polyurethane, polyolefins (such as polyethylene or polypropylene), polyvinyl chloride, polyvinyl acetal, cellulose acetate, polyvinyl chloride, polyvinyl acetal, cellulose acetate, polyvinyl acetate, polystyrene, polymethyl acrylate, polymethyl methacrylate, polyacrylonitrile, thermoplastic polyesters, polyvinyl alcohol, and gelatin; and thermosetting resins such as thermosetting polyesters, epoxy resins, and melamine resins.

As is conventional in the art, additives such as plasticizers, fillers, lubricants, stabilizers, antioxidants or mold releasing agents may be added as needed to the resin in order to improve its moldability, storage stability, plasticity, tackiness, lubricity, etc.

Examples of the plasticizers are dioctyl phthalate, dibutyl phthalate, dicapryl phthalate, dioctyl adipate, diisobutyl adipate, triethylene glycol di(2-ethyl butyrate), dibutyl sebacate, dioctyl azelate, and triethylhexyl phosphate, which are generally used as plasticizers for resins. The amount of the plasticizer can be varied over a wide range according, for example, to the type of the resin and the type of the plasticizer. Generally, its 100 parts by weight, per 100 parts by weight of the resin. The optimum amount of the plasticizer is not more than 80 parts by weight per 100 parts by weight of the resin.

Examples of fillers are fine powders of calcium oxide, magnesium oxide, sodium carbonate, potassium carbonate, strontium carbonate, zinc oxide, titanium oxide, barium sulfate, lithopone, basic magnesium carbonate, calcium carbonate, silica, and kaolin. They may be used either alone or as mixtures of two or more.

The amount of the filler is not critical, and can be varied over a wide range according to the type of the resin, the type of the filler, etc. Generally, the amount is up to 1000 parts by weight, preferably not more than 500 parts by weight, more preferably up to 200 parts by weight.

Usually its thickness is at least 3 microns. The upper limit of the thickness is neither strict, but is advantageously set at 100 microns for the reason stated above. Preferably, the thickness is 5 to 60 microns, more preferably 10 to 40 microns.

The semiconductive resin layer 4 laminated on the support layer is broken by discharging. It has a surface resistance of 10 to  $10^9$  ohms, preferably  $10^3$  to  $10^7$  ohms, more preferably  $10^4$  to  $10^6$  ohms and a volume resistance of 1 to  $10^6$  ohms-cm, preferably 10 to  $10^5$  ohms-cm, more preferably 10 to  $10^4$  ohms-cm.

The semiconductive resin layer 4 can be formed by dispersing a conductivity-imparting agent in a resin matrix.

The resin matrix forming a substrate for the semiconductive resin layer 4 may be chosen from those which have been described hereinabove about the non-recording layer composed of a metal powder-containing resin. The thermoplastic resins are especially suitable, and polyethylene, cellulose acetate and polyvinyl acetal are used advantageously. As needed, the resin may contain additives of the types described hereinabove such as plasticizers and fillers in the amounts described.

When a filler having a different conductivity from the conductivity-imparting agent, generally having a lower

conductivity than the conductivity-imparting agent, is included in the semiconductive resin layer 4, the breakdown of the semiconductive resin layer 4 by electric

discharging may occur more sharply. Suitable fillers of this kind are fine powders of inorganic substances such as magnesium oxide, calcium oxide, sodium carbonate, potassium carbonate, strontium carbonate, titanium oxide, barium sulfate, lithopone, basic magnesium carbonate, calcium carbonate, silica, kaolin clay, and zinc oxide. They can be used singly or as a mixture of two or more.

Of these, titanium oxide and calcium carbonate are especially suitable. The average particle diameter of the filler is generally 10 microns at most, preferably not more than 5 microns, more preferably 2 to 0.1 microns.

The amount of the filler can be varied over a wide range according to the type of the resin, etc. The suitable amount is generally 10 to 2,000 parts by weight, preferably 20 to 1,000 parts by weight, more preferably 50 to 400 parts by weight, per 100 parts by weight of the resin.

The conductivity-imparting agent to be dispersed in the resin to impart semiconductivity may be any material which has conductivity and gives the surface resistance and volume resistance described above to the resin layer. Generally, suitable conductivity-imparting agents have a specific resistance, measured under a pressure of  $50 \text{ kg/cm}^2$ , of not more than  $10^6 \text{ ohms-cm}$ . Examples of such a conductivity-imparting agent include carbon blacks; metals such as gold, silver, nickel, molybdenum, copper, aluminum, iron and conductive zinc oxide (zinc oxide doped with 0.03 to 2.0% by weight, preferably 0.05 to 1.0% by weight, based on the zinc oxide, of a different metal such as aluminum, gallium, germanium, indium, tin, antimony or iron); conductive metal-containing compounds such as cuprous iodide, stannic oxide, and metastannic acid; and zeolites.

Of these, carbon blacks, silver, nickel, cuprous iodide, conductive zinc oxide are preferred, and carbon blacks and conductive zinc oxide are more preferred. The carbon blacks which also act as a coloring agent are most preferred.

Carbon blacks differ somewhat in conductivity according to the method of production. Generally, acetylene black, furnace black, channel black, and thermal black can be used.

The conductivity-imparting agent is dispersed usually in the form of a fine powder in the resin. The average particle diameter of the conductivity-imparting agent is 10 microns at most, preferably not more than 5 microns, especially preferably 2 to 0.005 microns. When a metal powder is used as the conductivity-imparting agent, it is preferably in a microspherical, dendric or microlumpy form. Moreover, since a resin sheet having the metal powder dispersed therein tends to be electrically aniso-

tropic if its particle diameter exceeds 0.2 micron. Hence, the particle size of a metal powder in the above-mentioned form to be used as a conductivity-imparting agent for the semiconductive resin layer 4 or the conductive layer 6 should be at most 0.5 micron, preferably not more than 0.2 micron, more preferably 0.15 to 0.04 micron. Scale-like or needle-like powders can also be used, but should be combined with powders of the above forms.

The amount of the conductivity-imparting agent to be added to the resin can be varied over a very wide range according to the conductivity of the conductivity-imparting agent, etc. The amount is that sufficient to adjust the surface resistance and volume resistance of the semiconductive resin layer 4 to the above-mentioned ranges. For example, carbon blacks are incorporated generally in an amount of 1 to 300 parts by weight, preferably 2 to 200 parts by weight, more preferably 3 to 150 parts by weight, per 100 parts by weight of the resin. The other conductivity-imparting agents are used generally in an amount of 3 to 500 parts by weight, preferably 5 to 400 parts by weight, more preferably 10 to 300 parts by weight, per 100 parts by weight of the resin.

The thickness of the semiconductive resin layer 4 is not critical, and can be varied over a wide range according to the uses of the final product, etc. Generally, its thickness is at least 2 microns, preferably 3 to 50 microns, more preferably 5 to 20 microns.

According to the present invention, the conductive layer 6 is laminated on the other surface of the semiconductive resin layer 4.

The conductive layer 6 plays an important role in performing electric discharge breakdown with high accuracy by converging the current flowing through the semiconductive resin layer at a point immediately downward of the electric discharge recording stylus. The conductive layer 6 has a surface resistance of not more than  $10^4$  ohms, preferably not more than  $5 \times 10^3$  ohms, more preferably  $10^{-1}$  to  $2 \times 10^3$  ohms and a volume resistance of not more than  $10^2$  ohms-cm, preferably not more than 50 ohms-cm, more preferably not more than 20 ohms-cm.

The conductive layer 6 having such resistance characteristics may be a conductive resin layer comprising a thermoplastic or thermosetting resin and a conductivity-imparting agent dispersed in it, a vacuum-deposited metal layer, or a metal foil layer.

The thermoplastic or thermosetting resin that can be used in the conductive resin layer can also be selected from those described hereinabove in connection with the non-recording layer. Of these, the thermoplastic resins, especially polyethylene, cellulose acetate and polyvinyl acetal, are used advantageously. The conductivity-imparting agent to be dispersed in the resin may be chosen from those described above in connection with the semiconductive resin layer. Carbon blacks and metal powders are especially suitable. Carbon blacks are particularly preferred over metals in view of cost factors.

The conductivity-imparting agents are added in amounts which will cause the resin layer to have the electrical resistance characteristics described above. The amounts vary greatly according to the type of the conductivity-imparting agent. For example, carbon blacks are used in an amount of generally at least 10 parts by weight, preferably 20 to 200 parts by weight, more preferably 30 to 100 parts by weight; the other

conductivity-imparting agents especially metal powders, are used in an amount of at least 50 parts by weight, preferably 100 to 600 parts by weight, more preferably 150 to 400 parts by weight, both per 100 parts by weight of the resin.

As needed, the conductive resin layer may contain the aforesaid additives such as plasticizers and fillers in the amounts stated.

The thickness of the conductive resin layer is not critical, and can be varied widely according to the uses of the final products, etc. Generally, it is at least 3 microns, preferably 3 to 50 microns, more preferably 5 to 20 microns.

The conductive layer 6 may be a vacuum-deposited metal layer. Specific examples of the metal are aluminum, zinc, copper, silver and gold. Of these, aluminum is most suitable.

The thickness of the vacuum-deposited metal layer is neither restricted strictly. Generally, it is at least 4 millimicrons, preferably 10 to 300 millimicrons, more preferably 20 to 100 millimicrons. By an ordinary vacuum-depositing method for metal, it can be applied to one surface of the semiconductive resin layer 4.

The conductive layer 6 may also be a thin metal foil, for example an aluminum foil. It can be applied to one surface of the semiconductive resin layer 4 by such means as bonding or plating.

It is understood that at least one of the layers 4 and 6 may contain a coloring substance. Useful coloring substances are carbon black, inorganic and organic pigments, and dyes.

Carbon black has superior conductivity and acts both as a coloring substance and a conductivity-imparting agent as stated above. Thus, when the semiconductive resin layer or the conductive resin layer already contains carbon black as a conductivity-imparting agent, it is not necessary to add a further coloring substance. The inclusion of other suitable coloring substance is of course permissible.

Examples of pigments other than carbon black include inorganic pigments such as nickel yellow, titanium yellow, cadmium yellow, zinc yellow, ochre, cadmium red, prussian blue, ultramarine blue, zinc white, lead sulfate, lithopone, titanium oxide, black iron oxide, chrome orange, chrome vermillion, red iron oxide, red lead and vermillion, and organic pigments of the phthalocyanine, quinacridone and benzidine series such as aniline black, naphthol yellow S, hanza yellow 10G, benzidine yellow, permanent yellow, Permanent Orange, Benzidine Orange G, Indanthrene Brilliant Orange GK, Permanent Red 4R, Brilliant Fast Scarlet, Permanent Red F2R, Lake Red C, Cinquasia Red Y (Dup) (C.I. 46500), Permanent Pink E (FH) [Quido Magenta RV 6803(HAR)], and Phthalocyanine Blue (C.I. Pigment Blue 15).

Examples of useful dyes are azoic dyes, anthraquinone dyes, thionidigo dyes, quinoline dyes, and indanthrene dyes.

The pigments and dyes described are used either alone or in combination according to the color desired to be formed on a transfer recording sheet.

The amount of the pigment or dye can be varied over a wide range according to the type, color intensity, etc. of the coloring substance. Generally, it is at least 1 part by weight, preferably 2 to 1,000 parts by weight, more preferably 3 to 500 parts by weight, per 100 parts by weight of the resin.

When the pigment or dye is to be incorporated in both of the semiconductive resin layer 4 and the conductive resin layer 6, it is desirable that pigments or dyes be of an identical color or have colors of the same series.

The composite electric discharge transfer material of this invention can be formed by known methods, for example a melt-extrusion method, a melt-coating method, a melt-calendering method, a solution casting method, an emulsion casting method or combinations of these methods.

The composite electric discharge recording material of this invention described above is useful as an electric discharge transfer recording material or an electric stencil master sheet.

The electric discharge transfer recording mediums of the present invention are generally employed by superimposing the transfer recording medium onto a recording sheet 8, e.g., cellulosic paper, a synthetic paper-like sheet or a plastic sheet so that the conductive layer 6 contacts recording sheet 8. When electric discharge recording is performed by a discharge recording stylus in accordance with an ordinary method from the side of the graphite powder-containing resin layer 2, the semiconductive resin layer 4 and the conductive layer 6 are simultaneously broken by electric discharging, and the broken pieces 10 are transferred to the record sheet and fixed thereon, thereby achieving transfer recording.

It is understood that the electric discharge transfer film of this invention can be processed to any desired width or length in accordance with its desired use. For example, the transfer film can be used in the form of a narrow tape, such as a typewriter ribbon.

In electric discharge recording, the semiconductive resin layer and the conductive layer of the composite electric discharge transfer recording material are broken down, but the conductive (metal, graphite or carbon) powder-containing resin layer 2 is not broken because of its electric anisotropy and remains substantially unchanged. Accordingly, dissipation of any offensive odor issued at the time of electric discharge breakdown is inhibited, and soot or a coloring substance such as carbon black is prevented from scattering and adhering to the discharge recording stylus. The troublesome inspection and maintenance of the discharge recording stylus can be markedly reduced, and recording can be performed with high reliability. The term "electrical anisotropy" refers to the low resistance of support layer or conductive powder containing resin layer 2 in the through direction and the high resistance of this layer in the lateral direction.

The use of the composite electric discharge recording material can afford a sharp recorded image, and in electric discharge transfer recording, a transfer recorded image having a high density, a natural appearance and a soft tone can be obtained.

The composite electric discharge recording material of this invention can be used a plurality of times.

The composite electric discharge recording material of this invention can be conveniently used in facsimile systems, terminal recording devices in electronic computers, automatic recording devices of automatic measuring instruments, and various types of printers, etc.

The following examples further describe the present invention.

### EXAMPLE 1

A transfer sheet in accordance with this invention was prepared as follows.

5 A stock solution (A-1) containing 13.75 grams ES-TANE 5715 (polyurethane) sold by B. F. Goodrich Co., 13.75 grams of a phenoxy resin used in accordance with this invention and sold as PKHH by Union Carbide Corporation, and 72.5 grams methyl ethyl ketone was mixed together and stirred until complete dissolution was achieved. A second solution containing 10 grams of particulate graphite, sold as Micro 650 by Asbury Graphite, 90 grams resin solution, 40 grams methyl ethyl ketone, and 2.1 grams Byk Special sold by Mallinckrodt Chemical Company, was blended with the first solution in a chilled Waring blender for 15 minutes and then allowed to settle for 15 minutes.

The resulting solution was coated on a release sheet with a gap coated to a dry thickness of 1.1 mils, air dried for 5 minutes and then dried in a oven at 65° C. for 15 minutes.

20 Another solution (B) was prepared by introducing 22.5 grams ELVACITE 2044 (poly-n-butyl methacrylate) sold by E. I. du Pont de Nemours & Co., and 74.4 grams TOLUSOL 25, sold by Shell Chemical Company, into an 8 oz. plastic bottle. The bottle was rolled on a jut null until the contents were dissolved. 7.5 grams Black Pearls L which is carbon black, sold by Cabot Corporation, and 600 grams of 1" stainless steel (Type 25 440) shot was added to the solution and the same was milled for 16 hours. The resulting soluiton was coated over the first coating to a dry thickness of 0.5 mil using a Mayer rod (about #22). The product was oven dried at 65° C. for 3 minutes.

30 A final solution (C-1) was prepared by introducing 25.0 grams Aquadag E (graphite dispersion, 22% solids in water) and 75.0 grams ethanol in an 8 oz. bottle. The contents were stirred rapidly for 60 minutes with vortex blades. This solution was coated over the second coating (from solution B) to a dry thickness of 0.3 mil using a Mayer rod (about #18),and oven dried at 65° C. for 3 minutes.

### EXAMPLE 2

45 A transfer sheet was prepared in accordance with Example 1 except that a solution (C-2) containing 25.0 grams AQUABLACK 548-17 (24% carbon black in water) or 428-238, sold by Borden Chemical Co., 2.0 grams Rhoplex P-376 (acrylic resin dispersion in water, 50% solids) and 27.0 grams water was substituted for solution C-1 and processed in the same manner as solution C-1.

50 In the present specification, the terms "surface resistance" and "volume resistance" are determined in accordance with the method described by H. R. Dalton in U.S. Pat. No. 2,664,044.

55 According to a further embodiment of the present invention, a color coupler may be put in one or more transfer layers to react with a material in the recording material or paper, to generate a colored image, e.g., bis phenol A and leuco dye.

60 In the detailed description of the present invention, a transfer film comprising a support layer and two transfer layers is disclosed. It is understood that the present invention also encompasses the use of a support layer, as disclosed herein, having only one or possibly more than two transfer layers as disclosed herein provided that at least one of the transfer layers is thermally or electro-

thermally transferable to another substrate, e.g., a paper sheet. The nature of these transfer layers are discussed herein.

What is claimed is:

1. An electric discharge transfer material comprising:
  - (a) an electrically anisotropic support layer having electroconductive particles dispersed in a resin; and
  - (b) at least one thermal or electrothermal transfer layer in the form of a resin layer capable of being broken by electrical discharge and transferred to a record sheet, one of said transfer layers being laminated to said support layer, the improvement wherein said resin in the support layer comprises a phenoxy resin of the formula:



wherein n is about 100.

2. The electric discharge transfer material of claim 1 wherein said phenoxy resin has a molecular weight 25 20,000 to 30,000.

3. The electric discharge transfer material of claim 2 wherein said electroconductive particles are graphite 30 particles having a particle size between 0.1 and 20 microns.

4. The electric discharge transfer material of claim 3 wherein said support layer contains between 5 to 65% by weight graphite, based on the weight of the resin. 35

5. The electric discharge transfer material of claim 4 wherein said support layer contains between 15 to 45% by weight graphite based on the weight of the resin.

6. The electric discharge transfer material of claim 5, wherein the semiconductive resin layer comprises a thermoplastic or thermosetting resin and carbon black and a filler dispersed therein. 40

7. The electric discharge transfer material of claim 3 wherein said support layer contains between 25 and 45

35% by weight graphite based on the weight of the resin.

8. The electric discharge transfer material of claim 7 wherein the particle size of said graphite is between 0.1 and 1 micron.

9. An electric discharge transfer material comprising:

- (a) a semiconductive resin layer capable of being broken by electric discharging which has a surface resistance of 10 to  $10^9$  ohms and a volume resistance of 1 to  $10^6$  ohms-cm;
- (b) an electroconductive particle-containing electrically anisotropic phenoxy resin layer wherein said resin is of the formula:



wherein n is about 100 and said resin layer is laminated on one surface of the semiconductive resin layer (a); and

- (c) a conductive layer having a surface resistance of not more than  $10^4$  ohms and a volume resistance of not more than  $10^2$  ohms-cm, which is laminated on the other surface of the semiconductive resin layer.

10. The electric discharge transfer material of claim 9 wherein said electroconductive particles are graphite and said layer (b) contains between 5 to 65% by weight graphite, based on the weight of the resin.

11. The electric discharge transfer material of claim 10 wherein said layer (b) contains between 25 and 35% by weight graphite based on the weight of said resin.

12. The electric discharge transfer material of claim 11 wherein the particle size of said graphite is between 0.1 and 1 micron.

13. The electric discharge transfer material of claim 12 wherein at least one of the semiconductive resin layer (a) and the conductive layer (c) contains a coloring substance.

14. The electric discharge transfer material of claim 13 wherein the coloring substance is carbon black.

\* \* \* \* \*